

April 21, 1953

C. A. SNAVELY

2,635,993

ELECTROLYTIC PRODUCTION OF CHROMIUM HYDRIDE

Filed Oct. 16, 1948



INVENTOR.

Cloyd A. Snavely

BY

*W. B. Lilly*  
ATTORNEY

## UNITED STATES PATENT OFFICE

2,635,993

ELECTROLYTIC PRODUCTION OF  
CHROMIUM HYDRIDE

Cloyd A. Snavely, Columbus, Ohio, assignor, by  
mesne assignments, to The Battelle Develop-  
ment Corporation, Columbus, Ohio, a corpora-  
tion of Delaware

Application October 16, 1948, Serial No. 54,987

2 Claims. (Cl. 204—89)

1

This invention relates to a new method for making chromium hydride having a face-centered, cubic structure.

Metal hydrides have unusual and distinct properties which make them useful for numerous industrial and special applications. On being decomposed, they provide a source of chemically pure hydrogen which, released in the nascent or active atomic form, is highly reducing. This active hydrogen may be utilized to reduce the oxidized forms of metals to their metallic state, or to reduce various organic or inorganic compounds. After release of the hydrogen, the metal powder which remains is often in a very pure state. Furthermore, metal hydrides may be used in formulating compacts in powder metallurgy where the hydrogen released during subsequent sintering operations acts as a protective atmosphere to prevent oxidation.

The usual methods of producing metal hydrides have involved passing pure hydrogen gas through metal powder under carefully controlled conditions. These procedures have required a source of pure metal powder. Moreover, such methods have necessitated large supplies of hydrogen and extensive plant equipment for heating the metal powder and forcing the hydrogen gas through it. Certain of the metal hydrides which are not readily prepared by this method can be produced by reacting metal oxides with the hydrides of other metals which readily form hydrides.

The majority of the metal hydrides are relatively stable at ordinary temperatures, and to be decomposed they must be heated to elevated temperatures. This is a distinct disadvantage in those cases where it is desired to release active hydrogen, or to obtain fine, pure metallic particles, at low or moderate temperatures.

It is an object of this invention to provide a compound which is a source of active hydrogen and pure metal at low temperatures.

It is another object of this invention to provide face-centered, cubic, chromium hydride.

It is a further object of this invention to provide a process for making face-centered, cubic, chromium hydride.

It has been found that, if the current density and the concentration of chromium trioxide are maintained in a certain relationship, it is possible to plate face-centered, cubic, chromium hydride on a cathode from a low-temperature, aqueous chromic acid plating bath having an appreciable quantity of trivalent chromium ion therein and a high acid ratio.

The important relationship between the cur-

2

rent density and the concentration of chromium trioxide is illustrated by the figure where the concentration of chromium trioxide in grams per liter is plotted against current density in amperes per square foot. Outside of the band of the figure whose limits are defined by A and B, it has been found that only hydrolysis products, metallic chromium or hydrogen will be produced. In addition to maintaining this important relationship between the current density and the concentration of chromium trioxide, the bath must be operated at temperatures of from 0° C. to 25° C., have an acid ratio of from 250:1 to 350:1, and contain sufficient reducing agent to provide from 3% to 20% trivalent chromium ion in the bath from the reduction of hexavalent chromium ion.

A bath having a concentration of from 500 grams per liter of chromium trioxide to a saturated solution (about 1300 gms./l.) and operated at from 28 to 430 amps./sq. ft. will produce the hydride. Where the bath is operated at about 28 amps./sq. ft., the solution should be saturated with chromium trioxide, and less than 28 amps./sq. ft. at this concentration will not produce the hydride. On the other hand where the concentration of chromium trioxide in the bath is around 500 gms./l., the current density should be about 430 amps./sq. ft. At concentrations less than about 500 gms./l. of chromium trioxide, still higher current densities will not produce the hydride. The curve of the figure is shown as a broad band rather than as a narrow line to provide for slight variations in the bath composition and operating conditions which occur due to the temperature at which the bath is operated and the concentration of the reducing agent employed to reduce part of the hexavalent ion to the trivalent state. For example, if the process of plating is conducted where the concentration of chromium trioxide is 1000 grams per liter, the current density in the cell may vary from about 85 to about 145 amps. per square foot as indicated by the range defined by the points *a* and *b* on the band shown in the figure. In general, it has been found that, the other conditions of the plating process remaining constant (concentration of sulfuric acid, reducing agent, hexavalent chromium ion, trivalent chromium ion, and temperature), an increase in concentration of chromium trioxide requires a decrease in current density if face-centered, cubic, chromium hydride is to be plated on the cathode.

The sulfate ion concentration should be low, or conversely, the acid ratio ( $\text{CrO}_3/\text{SO}_4$ ) should be

high. Sufficient sulfuric acid should be added to the bath to give an acid ratio of from about 250/1 to 350/1. It is preferred to utilize a bath having a chromium trioxide to sulfate ion ratio of about 300 to 1. In place of the sulfuric acid, other compounds which furnish the  $\text{SO}_4$  radical and which do not adversely effect the electrolytic bath, may be employed. Suitable compounds of this nature are sodium sulfate, calcium sulfate, and chromium sulfate.

Trivalent chromium ions which are needed for the successful deposition of face-centered, cubic, chromium hydride from this electrolytic bath are obtained from the reduction of hexavalent chromium ions. It has been found that the bath should have a concentration of from 3% to 20% trivalent chromium ion for successful production of the hydride. To reduce the hexavalent ion to the trivalent state it is necessary to use a suitable reducing agent. Such reducing agents are well known in the art and it is only necessary that harmful by-products are not thereby introduced into the bath by cathodic reduction or by direct addition. Cane sugar has been found to be a very satisfactory reducing agent, as is hydrogen peroxide.

From about 5 to 40 grams of sugar per liter is satisfactory to reduce enough chromium to the trivalent state and to provide a sufficient concentration of the ion in the electrolyte. It is preferred to employ a concentration of sugar in the amount of from 10 to 20 grams per liter.

While the electrolytic process is being carried on, the bath should be maintained at a low temperature. The temperature of the bath should be held below 25° C. and above a temperature which would freeze the bath. Satisfactory deposits have been obtained when the bath temperature was between 0° C. and about 12° C. Excellent results have been achieved with a bath held at a temperature of between 2° C. and 8° C.

Insoluble anodes are best for use in plating the hydride. Antimonial lead anodes are preferred as they are easily obtained and are satisfactorily inert. Pure lead or iron anodes may be used but are less satisfactory, because both are less inert than lead alloy anodes to the chemical environment prevailing in the bath. Iron anodes also seem to lack the desirable properties associated with the lead oxide coatings formed on lead or lead alloy anodes during electrolysis of the bath.

The cathode on which the hydride is plated may consist of copper, brass, steel, or any of the metals which are commonly plated with metallic chromium.

The plating time is not believed critical, for it only determines the thickness of the deposit on the cathode. Some plates have been produced in a few minutes. Thick deposits were obtained after the process had been carried on for several hours.

The hydride deposited on the cathode is taken directly from the plating bath with no anodic replenishment. Periodic additions of chromium trioxide to the bath are therefore necessary. The sulfate concentration of the bath is not similarly reduced, the only appreciable losses of this constituent being the amount removed from the bath in the solution film clinging to the plated work. Such losses are referred to as dragout losses. Periodic checks are necessary to keep the acid ratio within the desired limits.

The following examples are set forth to more readily enable those skilled in the art to practice the invention:

#### Example 1

One thousand grams of chromium trioxide were dissolved in a liter of water. 3.3 grams of sulfuric acid were then added and mixed into the solution. 20 grams of cane sugar in the form of an aqueous syrup were then slowly added to this solution. A strong reaction proceeded, the sugar reducing much of the chromium, which was in the hexavalent state, to the trivalent state. After the reaction had subsided the bath was tested or titrated, and it was found that the trivalent chromium content of the bath was now approximately 12% of the total chromium present. The electrolytic bath was then refrigerated to 5° C., plus or minus 4 degrees. Electrodes of lead and copper were then placed in the bath, the anode being lead and the cathode being copper. An electric current was then passed through the electrolytic bath which was sufficient to create a current density in the cell of 115 amps per square foot. After seven hours a deposit on the cathode was obtained which was dark gray and lustrous in color and extremely scratch resistant. On X-ray analysis it was found to have a face-centered, cubic structure. Chemical and physical analyses were performed on this deposit which showed that it contained only chromium and hydrogen.

#### Example 2

A solution was prepared similar to that shown in Example 1 containing 911 grams per liter of chromium trioxide and sufficient sulfuric acid to give a 300:1 acid ratio. 10 grams per liter of cane sugar were added to this bath. On titrating it was found that approximately 5% of the chromium was reduced to the trivalent state. Samples plated from this bath at temperatures below 5° C. and at a current density of approximately 115 amps per square foot over a 17-hour interval were X-rayed. The X-ray data showed this material to also have a face-centered, cubic structure. Further analysis of the deposit showed that it contained chromium and hydrogen.

This process used to plate face-centered, cubic, chromium hydride may be adjusted by changing the concentrations of ingredients or conditions within the ranges indicated so that the resulting plate is dull gray, black, or lustrous black in appearance.

Table 1, below, gives the X-ray data obtained by experiment and calculation. X-ray equipment used in obtaining the experimental data was a X-ray spectrometer as described by Friedman in "Electronics," April 1945, page 132. Approximately 250 samples of plate were produced during this investigation and most of these were X-rayed from 1 to 10 times to identify their initial structures and any structural changes occurring after the initial determination.

TABLE 1

| Sample                                | Cu Radiation- $2\theta$ (in Degrees) |      |       |      |      |      |      |
|---------------------------------------|--------------------------------------|------|-------|------|------|------|------|
|                                       | 40.7                                 | 44.4 | 47.25 | 64.6 | 68.8 | 83.1 | 87.2 |
| Body-centered cubic chromium          | X                                    |      |       | X    |      |      |      |
| Face-centered cubic, chromium hydride | X                                    |      | X     |      | X    | X    | X    |
| Sample as plated                      | X                                    | X    |       | X    | X    | X    | X    |
| Sample after heating                  | X                                    |      | X     |      |      |      |      |

1. Values of  $2\theta$  for B. C. C. structure were calculated from established lattice constants.  $2\theta$  values for F. C. C. structure are experimental values obtained in the present work.

2. "Heating" consisted in placing samples in an oven held at 150° C. for an hour to decompose the hydride structure.

From these dimensions it was possible to compute the lattice parameter of the face-centered, cubic structure which was found to be  $a_0=3.85$  angstrom units. The distances between centers of adjacent chromium atoms was also computed for this structure and found to be approximately 2.712 angstrom units. The lattice parameter, however, of body-centered, cubic chromium is given in the literature as  $a_0=2.87$  (6) Å, and the distance between centers of adjacent atoms is 10 2.492 (9) Å.

Hydrogen atoms are believed to occupy the second largest openings in the lattice. Metal-hydrogen combinations of the general formula  $MH$  to  $MH_2$  crystallize in the face-centered, cubic atomic arrangement with metal atoms at the normal corner and face-centered positions of the unit cell. The hydrogen atoms then occupy half of the second largest interstitial openings to form a zinc blende type of structure for the formula  $MH$  as proposed for alloys by Westgren, "Jnl. Franklin Inst.", 212 (1931) 577, or all of the second largest interstitial openings to form a fluorite type of structure for the formula  $MH_2$ , also as proposed by Westgren.

The atomic radius of chromium in the body-centered cubic arrangement is  $1.24+A$ , and the Goldschmidt correction, "Z. Physikal. Chem.", 133 (1928) 397, applied to this requires a radius of  $1.28+A$  for atomic arrangements of coordination number 12. If atoms of radius  $1.28+A$  are considered to be the metal atoms in a face-centered, cubic lattice of parameter 3.85 Å, the largest opening in the structure is at the center of the unit cube. This opening is 1.29 Å, in smallest diameter. The second largest openings are 0.78 Å, in smallest diameter and are centered on positions in the unit cube of  $\frac{1}{4} \frac{1}{4} \frac{1}{4}$ , and the seven corresponding positions in the lattice. The diameter of the interstitial hydrogen atoms in face-centered, cubic structures is given in the literature as being between 0.80 Å and 1.00 Å. A hydrogen atom of this size accounts for the lattice parameter of the face-centered, cubic, chromium plate. Thus, the face-centered, cubic plate is in reality a hydride of the zinc blende type of structure. Since the fluorite type structure is only a more filled-up version of the zinc blende structure, it is likely that any combination of chromium-hydrogen atoms from 50 atomic per cent Cr—50 atomic per cent H (zinc blende type) to 33 atomic per cent Cr—67 atomic per cent H (fluorite type) should be possible.

To provide further proof that the face-centered cubic, chromium plates were hydrides, some hydrogen extraction tests were undertaken. A sample of face-centered, cubic, chromium hydride plate was produced from a bath containing 1021 grams per liter of chromium trioxide having a 300:1 acid ratio, and with 7.4 per cent of the total bath chromium in the trivalent state from the reduction of hexavalent chromium ion by 20 grams per liter of cane sugar. The bath temperature was approximately 0° to 4° C., the current density was 115 amps. per sq. ft., and the plating time was 7½ hours. The backing for this plate was copper foil, 0.002-inch thick. Upon removal from the plating bath, the sample was quickly rinsed, sponged dry with a towel and placed under mercury in an inverted test tube. This operation required approximately two minutes. Gas was evolved from the specimen for less than twenty-four hours at an appreciable rate; no further cold evolution being noted in three days. The sample was then transferred to a gas 70 75

extraction apparatus where it was heated to 650° C. and held at this temperature for 30 minutes while under a vacuum. The gas extracted by this treatment and from the cold evolution was analyzed and found to be pure hydrogen. Calculated at standard temperature and pressure, the cold evolution gas had a volume of 1.41 ml., and the warm extraction gas had a volume of 10.80 ml., giving a total gas content of 12.21 ml. for the sample. This amount of hydrogen was considered to be evolved entirely from the chromium plate, as previous experience has shown that a negligible amount of hydrogen may be held in a copper disc measuring only  $\frac{1}{2}$  inch in diameter and 0.002 inch in thickness. The apparatus used to extract the hydrogen gas was similar to that described by Newell, "Journal of the Iron and Steel Institute," 141 (1940), 243.

The copper backing was stripped off the sample in nitric acid and the residue was weighed. It was then treated with hydrochloric acid which dissolved some of the chromium. The undissolved residue was a green powder, and it was concluded that it was chromic oxide ( $Cr_2O_3$ ) which was then fused with potassium bisulfate, some residue remaining. A sodium peroxide fusion treatment served to dissolve this residue. The entire lot of dissolved chromium was then oxidized with sodium peroxide and titrated by the iodine-thiosulphate method, from which the amount of chromium in the sample was found to be 0.0329 gram. Since the weight of the sample was 0.0511 gram, it is evident that roughly half of the sample was in the form of chromic oxide ( $Cr_2O_3$ ) after the high-temperature extraction treatment.

The chromium atom to hydrogen atom ratio calculated from the above data is 1:1.7. This result entirely agrees with the expectations, as a chromium:hydrogen ratio anywhere within the limits of 1:1 and 1:2 would satisfy the requirements previously computed with X-ray data for the face-centered, cubic structure. It is, therefore, believed that face-centered, cubic, chromium hydride has the general formula  $CrH_{(1+N)}$ , wherein N ranges from 0 to 1.

In summary this invention discloses a new and novel process for plating chromium hydride on a cathode from a low temperature chromic acid bath, containing a minor amount of sulfuric acid and an appreciable quantity of trivalent chromium ion, by maintaining a definite relationship between the chromium trioxide and the current density. This relationship is indicated by the shaded area of the curve defined by the limits A and B, of the figure. In general, within the ranges indicated, the current density will vary inversely with the concentration of chromium trioxide in the bath. The method disclosed herein is extremely easy to perform and does not demand the use of involved techniques nor complicated machinery as compared to known processes for manufacturing other metallic hydrides. Furthermore, face-centered, cubic, chromium hydride which is produced by the method of this invention provides a ready source of nascent hydrogen for reducing or catalytic reactions at low temperatures unlike other metallic hydrides, for it has the property of decomposing slowly at atmospheric temperatures and rapidly at only slightly elevated temperatures. It is, however, brittle and may be subjected to comminution to produce a very fine powder which is highly suitable for use in making up

powder compacts; and it is also a source of pure, metallic chromium.

What is claimed is:

1. The method of producing essentially pure face-centered cubic, chromium hydride, which comprises passing an electric current from an anode to a cathode through an electrolytic bath at a temperature of from 0° C. to 12° C., said bath consisting of an aqueous solution of chromium trioxide, from 5 to 40 grams per liter of sugar, a sufficient amount of a compound furnishing the  $\text{SO}_4$  radical selected from the group consisting of sulfuric acid, sodium sulfate, calcium sulfate, and chromium sulfate to give a chromium trioxide to acid radical ratio of 300 to 1, while maintaining the current density of the cell from 105 to 125 amperes per square foot with the concentration of chromium trioxide in the substantially inverse ratio of 1100 to 900 grams per liter.

2. A composition of matter useful in the method of producing essentially pure face-centered cubic, chromium hydride, consisting of an aqueous solution of chromium trioxide, from 5 to 40 grams per liter of sugar, and a sufficient amount of a compound furnishing the  $\text{SO}_4$  radi-

10  
15

cal selected from the group consisting of sulfuric acid, sodium sulfate, calcium sulfate, and chromium sulfate to give a chromium trioxide to acid radical ratio of 300.1, the concentration of said chromium trioxide being from 900 to 1100 grams per liter.

5 CLOYD A. SNAVELY.

References Cited in the file of this patent

UNITED STATES PATENTS

| Number    | Name               | Date          |
|-----------|--------------------|---------------|
| 1,802,463 | Fink               | Apr. 28, 1931 |
| 1,842,535 | Brode et al.       | Jan. 26, 1932 |
| 1,967,789 | Sohn               | July 24, 1934 |
| 2,410,242 | Schulein           | Oct. 29, 1946 |
| 2,461,661 | Schlesinger et al. | Feb. 15, 1949 |

OTHER REFERENCES

20 Makariewa et al., *Zeitschrift für Elektrochemie*, vol. 41 (1935), pp. 623-631.

Wood, London, Edinburgh and Dublin Philosophical Magazine and Journal of Science, vol. 12 (1931), pp. 853-864; vol. 24 (1947), pp. 772-776.

25 Snavely, *Transactions of the Electrochemical Society*, vol. 92 (1948), pp. 541-545.